

No. 749,053.

PATENTED JAN. 5, 1904.

C. J. GRIST.  
GOLF BALL, &c.  
APPLICATION FILED SEPT. 19, 1903.

NO MODEL.

Fig. 1.



Fig. 2.



Fig. 3.



Witnesses.

James L. Morris, Jr.

Robert Everett.

Inventor.

Charles J. Grist.  
By James L. Morris.  
Atty.

## UNITED STATES PATENT OFFICE.

CHARLES JAMES GRIST, OF APSLEY, BANSTEAD, ENGLAND.

## GOLF-BALL, &amp;c.

SPECIFICATION forming part of Letters Patent No. 749,053, dated January 5, 1904.

Application filed September 19, 1903. Serial No. 173,895. (No model.)

*To all whom it may concern:*

Be it known that I, CHARLES JAMES GRIST, consulting engineer, a subject of the King of Great Britain, residing at Apsley, Banstead, 5 in the county of Surrey, England, have invented certain new and useful Improvements in the Manufacture of Golf-Balls and Balls for Like Uses, of which the following is a specification.

10 This invention relates to the improved manufacture of balls for use in the game of golf or the like and is designed to produce a golf-ball possessing the requisite qualities of lightness, elasticity, and resilience, so that it may 15 be driven well and truly and yet possess sufficient toughness and strength to resist hard wear.

Referring to the accompanying drawings, forming a part of the application, Figure 1 20 shows a partly external view and partly sectional view of a ball. Fig. 2 is an external view of the core of such an improved ball, and Fig. 3 is a detail view piece of the india-rubber tape.

25 *a* indicates the solid core, *b* the india-rubber tape, and *c* the external shell or cover.

In carrying out my invention I take linseed or other drying oil and heat it up to at least 400° Fahrenheit, adding litharge or other suitable 30 drying agent, taking care that it does not boil continuously for more than six hours at any one time, the whole of which time the oil is kept continuously in motion by suitable apparatus. I then take a fibrous substance— 35 such as hemp, jute, cotton, suitable animal fiber, or other fibrous substance suitable for the purpose—and subject the fibers to a cleaning process, such as carding. The fibers now are spread and subjected to a drying process, such as by means of heated air propelled or drawn through them, in order to remove as much as possible any trace of aqueous moisture. The oil having regained its normal 40 temperature, I take the fibers which have been treated as above described and immerse them in such oil, immediately removing them and placing them in a hydro extractor or other suitable machine for the purpose of extracting as much as possible all the superfluous oil, which is then drained away and may be used again. The fibers will now be found to have small globules of partially-oxidized oil

adhering at intervals on each fiber. These coated fibers being now in a somewhat matted condition from the previous treatment are 55 pulled apart and thoroughly loosened by the aid of suitable opening mechanism, such as a carding-machine. Then the fibers are spread loosely on wire gauze or netting and a current of heated air is made to pass through them by 60 means of a fan or other suitable machine, and in order that all the globules of oil in the fibers may be brought into contact with the heated air as much as possible the fibers must be turned or redistributed in the netting about 65 every hour. By these means nearly every globule of oil adhering to the fibers is thoroughly oxidized and dried. When this is accomplished, I take the fibers and redip in the oil, and when taken out of the hydro extractor it 70 will be found that more globules of oil are adhering to the fibers in the vacant spaces in between the former and already-oxidized particles. I repeat the drying process. A third and last time I dip the fibers and proceed as 75 before. I find that it is not expedient to dip more than three times, because most of the fibers being covered with globules of oxidized oil, should another dip take place the unoxidized oil might coat and spread on the oxidized oil, and if this happens the drying process cannot be thorough, as the heated air would not be able to play upon the whole of the unoxidized oil, and, oxidation being imperfectly accomplished, the resulting material 80 would be worthless. The fibers are now placed in masticating or grinding rolls of different diameters, running at a high speed and worked till they assume a homogeneous condition. When thoroughly crushed, I place 85 the material in mixing-rolls and add from five per cent. to ten per cent. of powdered sulfur. Care must be taken that the material does not become too highly heated, and this may be prevented by continually stripping the material off the rolls by means of a knife or gage adapted for the purpose. When the sulfur is thoroughly mixed with the material, the material is taken out and placed in an inclosed vessel, and this vessel 90 is heated up to about 360° Fahrenheit, preferably by means of a vessel steam-jacketed all over. The material is then laid on trays, avoiding any heaping up of the matters that will in- 95

terfere with uniform access of the heat there-  
to. When the material has assumed a porous  
or dry consistency, it is taken out and again  
placed in the mixing-rolls and ten per cent.  
5 to seventy-five per cent. of gutta-percha or  
rubber or other suitable substance, to im-  
part to the material greater cohesion, te-  
nacity, and resiliency, or a mixture of such  
materials, can be added. When thoroughly  
10 mixed, the material is placed in suitable molds  
to be pressed into rod or other convenient  
shape or be passed through a squiring-ma-  
chine of the ordinary pattern for the same  
purpose. It can then be cut into pieces  
15 which are heated to soften them, and these  
pieces while in a soft state are placed in suit-  
ably-sized molds adapted for balls of any  
desired pattern and pressed into shape.  
These balls are then allowed to become thor-  
20oughly hardened and afterward painted with  
any suitable paint, if required. Alternatively  
these balls are made with a hollow center by  
adopting the following process, say, for golf-  
balls: I make a small hollow ball of the de-  
25 scribed material and of a diameter of, say,  
about one and one-eighth inches, using a cup-  
shaped mold, the hollow portion of which re-  
ceives sufficient material for the production  
with the aid of correspondingly - shaped  
30 plunger of about three - fourths of an inch  
diameter of a cup or half-ball. The material  
when heated or softened is then placed in the  
mold and the plunger being pressed centrally  
in a press a half-hollow ball will be made.  
35 Two of these halves can be united firmly to-  
gether to make one hollow ball by means of  
heating the edges and pressing them firmly  
together or by means of a suitable adhesive  
material. The hollow ball so made is then  
40 allowed to get cold and hard. The ordinary  
golf-ball mold is now brought into use and  
some more of the material is heated or soft-  
ened and is divided into two equal or nearly  
equal portions, one being placed in each half  
45 of the mold. The hard hollow ball is now  
placed in the center between these two por-  
tions of soft material, and care should be  
taken that no moisture is present. The mold  
can then be placed in the press and the fin-  
50 ished ball be pressed out and allowed to cool  
and harden, the whole forming one mass of  
like material with a hollow center, as the in-  
terior, cold, and hard hollow ball will resist  
the pressure and the superfluous soft mate-  
55 rial will be exuded from the mold.

I sometimes make the balls (say golf-balls)  
by molding a hard solid ball of the afore-  
said material (or any other suitable hard ma-  
terial) of about three-fourths of an inch in  
60 diameter, and then this solid central - ball  
core is covered with rubber tape or thin sheet-  
rubber stretched over it until the size is in-  
creased to about one and one-eighth inches and

this inserted centrally, as before described,  
in the outer cover. 65

The small central ball must be made of a  
hard and comparatively light material, such  
as described, in order that when the finished  
ball is hit the rubber ball or wrapping inside  
will be compressed upon it and not into it, 70  
and by this means the full resilient energy of  
the blow will be utilized in the drive. In a  
ball so constructed I embody a compressed  
hard core of prescribed composition larger  
and harder than the india-rubber elastic core 75  
referred to, and I use a thin vulcanized india-  
rubber-tape winding which has been vulcan-  
ized to the point requisite to enable it to retain  
its elasticity even after it has been wound  
upon the hard core in a condition of consid- 80  
erable tension.

A noticeable feature of my improved con-  
struction is the limited thickness of the vul-  
canized india-rubber-tape winding upon the  
enlarged hard core and within a substantial 85  
cover of the prescribed material.

When my improved ball is hit by the club,  
the outer cover will be compressed, and this  
compression will be conveyed to the rubber  
tape; but the core resists the compression and  
presents a fairly large surface of resistance.  
Now the extra distance that a filled ball will  
carry in comparison to a solid ball is caused  
by the sharp recovery after compression by  
the wound filling of india-rubber, and in my 95  
improved ball this recovery is very quick be-  
cause of such larger and harder core.

When the ball strikes the ground, the re-  
covery of form will tend to make the ball  
shoot forward and not upward. The result 100  
of this reaction is that the energy of the re-  
silient rubber in my improved ball is utilized  
to its fullest extent for the purpose of the  
"stroke," and the movement of the ball is  
found to be more under the striker's control 105  
and this, especially for "putting," is a great  
consideration.

Having now particularly described and as-  
certained the nature of my said invention and  
in what manner the same is to be performed, 110  
I declare that what I claim is—

A golf-ball comprising a spherical core  
formed of fibrous material, oxidized oil, a  
drying agent, sulfur and rubber treated and  
compounded in the manner and substantially 115  
in the proportions herein described, a wrap-  
ping of vulcanized rubber tape wound about  
said ball, and an outer shell or cover molded  
about the tape or wrapping.

In testimony whereof I have hereunto set 120  
my hand in the presence of two subscribing  
witnesses.

CHARLES JAMES GRIST.

Witnesses:

RICHARD ELY,  
ANDREW C. KNOELLER.